

J. A. HANLON.  
METHOD OF COATING METAL.  
APPLICATION FILED SEPT. 18, 1912.

1,156,995.

Patented Oct. 19, 1915.



Fig. 5



Fig. 4



WITNESSES:

O. E. Wright.

Albert L. Hyde.

INVENTOR.  
John A. Hanlon  
Fredk W. Ulster

ATTORNEY.

# UNITED STATES PATENT OFFICE.

JOHN A. HANLON, OF PITTSBURGH, PENNSYLVANIA, ASSIGNOR TO HANLON-GREGORY GALVANIZING COMPANY, OF PITTSBURGH, PENNSYLVANIA, A CORPORATION OF PENNSYLVANIA.

## METHOD OF COATING METAL.

1,156,995.

Specification of Letters Patent.

Patented Oct. 19, 1915.

Application filed September 18, 1912. Serial No. 721,080.

To all whom it may concern:

Be it known that I, JOHN A. HANLON, a resident of Pittsburgh, in the county of Allegheny and State of Pennsylvania, have 5 invented a new and useful Improvement in Methods of Coating Metal, of which the following is a specification.

This invention relates to a method of coating metal, and particularly to a method of 10 coating steel or iron with lead, zinc, or compositions thereof.

The object of the invention is to provide a method whereby strips of iron or steel may be provided with a very thin coating 15 of metal applied in such manner that the coating metal is spread very evenly and forced into the pores of the base material, to form a firm and secure bond or physical connection therebetween, to enable the coated 20 material to be bent or folded upon itself or at very sharp angles, without breaking, cracking, stripping or peeling of the coating metal.

In the drawings, which illustrate one embodiment of apparatus for carrying out the method, Figure 1 is a longitudinal sectional elevation through the coating tank with a scraping device therein; Fig. 2 is a plan view of the scraping device; Fig. 3 is a 25 transverse section on the line 3—3, Fig. 2, one of the levers being shown in dotted lines in raised position; Fig. 4 is a longitudinal section on the line 4—4, Fig. 2; and Fig. 5 is an enlarged longitudinal section on the 30 line 5—5, Fig. 2.

Although in the past attempts have been made to provide strips of steel or iron with a thin closely adhering coating of zinc or lead, or compositions thereof, which will 40 not crack, break or peel, this has never been accomplished successfully to my knowledge. In the case of lead it has commonly been found that it will not adhere to the surface of the steel or iron or, if it does adhere, then 45 only in blotches or spots and not continuously, while, in the case of zinc, it has always been necessary to run the strip or sheet through the bath of metal at such a slow rate of speed as will permit the base metal 50 to be brought up to the temperature of the bath before leaving the same, which rate of speed is so slow as to permit a comparatively thick coating of zinc to be deposited on the strip, the wiping or stripping rolls or other 55 devices commonly employed, and through

which the strip passes as it emerges from the pot, being unable to so materially reduce or thin and spread this thick coating that it will not peel or crack when the sheet or strip is bent at sharp angles.

By my invention I propose to immerse or submerge a strip in a bath of the coating metal, by passing it therethrough, and then, after it emerges from the bath of metal, applying scrapers to both sides of the strip, 60 said scrapers being of such type and so applied as to remove a very considerable portion of the adhering coating metal to thereby thin the same. Preferably the strip will be passed through the bath at a considerably 65 higher rate of speed than according to prior practice, thereby reducing the period during which it is submerged in the metal, and the amount of coating metal which will adhere thereto. The strip may also, if desired, be passed successively through a plurality of similar scrapers which, in turn, 70 will remove increments or additional portions of the coating metal. According to 75 this method the scrapers not only remove 80 from the base material a large proportion of the coating metal which has adhered thereto, but also by pressure applied thereto, 85 compact the coating, spread it, and force it into the pores of the base metal, thereby forming a very thin coating having a firm 90 physical bond or connection to the base material so that the finished product may be bent or folded either upon itself, or at very sharp angles, without breaking, cracking, 95 stripping or peeling. This product, I believe, has never before been successfully produced.

To carry out the method I employ an apparatus of suitable construction, one embodiment thereof being shown in the drawings. This comprises a suitable pot or kettle 1 which is of cast or plate iron or steel, which is mounted on a suitable foundation 2 and is filled or nearly filled with molten metal 3 which it is desired to coat upon the strips or sheets, and which may be kept in a molten condition by any suitable or preferred arrangement of heating apparatus. The molten metal 3 may either be 100 wholly zinc, wholly lead, or compositions of these two metals. Near one end of the pot is located a transverse bar or support 4 having upwardly extending offset end portions 4<sup>a</sup> resting on or embedded in the side walls 105 110

of the foundation 2, or bolted to the pot or kettle and upon which bar or support is carried one end of the scraping device.

The scraping device comprises a suitable frame 5, the two side members of which, at their forward ends, are provided with downwardly bent hooks 6 to hook over the transverse bar or support 4, which is preferably so disposed as to lie a short distance below the level of the molten metal 3 in the pot. At the rearward end of the frame 5 its side members form a pair of handles 7 which may be used to lift the scraping device from the pot and place it in position therein when desired. Between the side members 5 are transverse members 8, 8<sup>a</sup> to tie the frame together and make it rigid.

As shown in Fig. 2, the transverse members 8, of which two or more may be used, as desired, are located near the forward end of the frame 5 and in such position as to be above the surface of the molten metal within the pot. These transverse members each carry a pair of oppositely disposed sets of scrapers or wiping devices, thus making four sets of such devices in all, although more may be used, if desired. Since all of the sets of scraping devices are alike, it will be necessary to describe only one thereof.

The scraping devices are preferably of the construction illustrated and claimed in my companion application Serial No. 721,079, filed September 18, 1912, and briefly described comprise a plate or support 12 secured to the transverse member 8, and having removably bolted thereto a lower scraping or wiping device 13, comprising a flat knife, blade or strip of rolled steel having either a square or rectangular upper edge portion, but preferably the latter, over which the strips of metal being coated pass through the apparatus. Above each of the scrapers 13 is mounted a co-operating upper scraping device 14, which is removably bolted to a supporting member 15, and which is of the same construction as the lower scraping device. The support 15 is pivotally secured at 11<sup>a</sup> to the upper end of a pivot member 11 vertically adjustable in a supporting ledge 10 on the frame, and, at its outer end, is provided with an upwardly offset handle member 16 to enable it and the upper scraping device to be raised from or lowered upon the strips passing through the device. It will also be understood that the handle member 16 moves between guides 18 on the frame and may be as long or as short as desired and may also be provided with suitable means, such as an aperture 17, for the attachment of a weight 17<sup>a</sup> thereto. The pot 1 is first filled with metal 3, such as zinc, lead, or both, which is heated to a molten condition suitable for coating metal therewith. The frame 5 being placed in position, one end of a strip 20 of steel or

iron, and supplied in the form of a coil, is passed between the upper and lower scraping knives of the first pair and then, in a similar manner, between the upper and lower scrapers of the second and succeeding pairs. The coil is supported on a suitable spindle and the free end of the strip is led to a suitable coiling or winding apparatus of the usual drum construction. This is then operated to wind up the strips and draw them through the bath of molten metal. The handle levers 16 which support the upper scrapers 14 are either themselves made of some weight, or have extra weights applied thereto, as stated, so that they press the upper scrapers down into very close contact with the upper surface of the strip, whereby the sharp edges of the scrapers of the first set remove or scrape off a considerable portion of the surplus bath metal and dross from both sides of the strip passing through the apparatus, which drains into the melting pot 1. At the same time, the scrapers 13 and 14 of the first set spread compact and thin the coating metal and force it into the pores of the strip. The pressure applied to the levers carrying the upper scrapers causes them, and the lower scrapers as well, to compact the coating metal and positively force the same into the pores of the base material. After the strip has passed the first set of scrapers it passes through a second similar set which removes a second portion of the coating metal and thin and spread the same and force it more firmly into physical connection with the base metal. Additional sets of scraping devices may be used if desired, although in practice, I have found that two sets are sufficient.

In coating metal, as heretofore carried out, it has never been the practice to operate the winding or coiling apparatus, to cause the strip to travel at a speed faster than the rate of flow of the molten metal itself, the common speed being about 15 feet per minute. From experience it is found that molten lead or zinc will flow upon the surface of base metal at a given rate, which rate is never exceeded by the rate of travel of the strip or sheet through the bath. By my improved method the surplus coating metal may be forcibly removed at almost any rate of travel of the strip through the scrapers. Consequently the strip being coated can be passed through the apparatus at a very high rate of speed, say, for example, at a rate of 100 feet per minute, more or less. The scraping devices are placed comparatively close to, but at the same time are spaced away from, the surface of the molten metal bath and the strip reaches the scrapers before the metal has a chance to solidify or set to any appreciable extent. In the case of zinc it is found that steel or iron may be

- produced with a three per cent. coating on 23 gage, in other words, with a coating of three pounds of zinc to every hundred pounds of base material. This coating is 5 very considerably thinner than any that has heretofore been applied and steel or iron thus coated with a zinc or lead coating may be bent or folded, as described, without any 10 danger of the surface coating cracking, breaking or peeling. When the pot or kettle is filled with molten lead, it is found that the lead adheres to the surface of the base material, probably due to the high rate of speed at which this passes through the 15 apparatus, and is thinned and compacted and bound to the base material to form a thin coating therefor. At the same time the coating is continuous and uninterrupted and will not crack, break or peel.
- 20 What I claim is:—
1. The method of coating metal strips, consisting in passing the same through a bath of molten metal at a rate of speed faster than the natural rate of flow of the molten 25 metal on said strips at or near the bath, to wit, at a speed in excess of fifty feet per minute, and applying edged scrapers with material pressure to both sides of the strips
- and thereby scraping off the surplus molten metal and dross before it solidifies and 30 spreading and pressing the remaining thin coating into the pores of the base material to thereby form a firm bond or physical connection between the strip and coating metal.
2. The method of coating steel or iron 35 strips with softer metal, consisting in passing the same through a molten bath of the softer metal at a rate of speed faster than the natural rate of flow of the molten metal on said strips at or near the bath, to wit, at 40 a rate of speed in excess of fifty feet per minute, and after it has left the bath and before the molten metal has left the strip forcibly scraping both sides of the strip to thereby remove the surplus coating metal 45 and dross before it solidifies and spread and thin the remaining coating and force it into the pores of the strip to thereby form a firm physical bond or connection therewith and a thin permanent coating for the same.
- 50 In testimony whereof, I have hereunto set my hand.

JOHN A. HANLON.

Witnesses:

ELBERT L. HYDE,  
J. L. TREFALLER, JR.